

## UNITED STATES PATENT OFFICE.

HENRY E. JODOIN, OF INDIAN ORCHARD, MASSACHUSETTS.

## COATING FOR SCREENS AND THE LIKE.

No Drawing.

Application filed May 15, 1924. Serial No. 713,618.

In the projection of photographic pictures and particularly in the so-called "moving picture" the screen or surface of display has presented a problem of considerable difficulty.

This problem is variously complicated by the material of the receiving surface and by its treatment. Taking for example the usual "drop"—in such we have a fabric 10 usually rolled and unrolled with considerable frequency and subjected to the widest variety of use and abuse.

When it is considered that the physical intercept of a figured beam of light involves 15 an infinitely varied problem of absorption and reflection, it is readily appreciated that the character of the surface is one of supreme importance. The usual "picture" as displayed is uncolored but I have discovered 20 that even in such the factor of color must be taken into account. In the case of colored displays the screen factor is of even more importance. For the sake of simplicity, however, I will discuss my invention in 25 connection with the uncolored picture or at least as it is generally so considered.

All sources of projection illumination 30 emit light more or less colored. Furthermore, films or other photographic "pictures" are taken from objects or surroundings variously colored. My invention therefore contemplates the introduction of color factors in the screen surface as a means of 35 reproducing the various qualities of the picture inherently present but heretofore undeveloped.

Reverting directly to the substance of my 40 invention, I have selected as illustrative thereof a specific application which is direct and applicable and yet serves to show to those skilled in the art those principles upon which my invention is founded.

By the way of example, I will take the 45 problem of surface coating an ordinary screen or drop of textile character. These are particularly susceptible to moisture which is another problem of the commercial moving picture house. Here is a continuously gathering constantly changing audience constantly admitting and introducing new factors of moisture and vapors which generally trend toward the proscenium arch or the screen plane. This introduces a factor of disintegration or at least 50 of tarnish on the screen. Briefly also there

is the factor of fire risk. Obviously the screen is a hazard or an element of safety.

I will therefore proceed to discuss my invention in the light of such suggested conditions. In accordance with my invention I 60 am able to treat any screen or drop in any ordinary state of repair or passable condition and bring it to relative perfection as follows:

I utilize a coating which may be variously 65 prepared but for simplicity and directness I disclose it in what seems to me its most direct and usable form.

For general use on any reasonably intact surface I prepare a coating for which the 70 following affords direction.

I prepare a coating for which in a small amount I utilize a calcareous base, as for example, five pounds of calcimine. Almost 75 any white mineral base will do, but I prefer to use one which is of a chalky character. This I wet up and work to a pasty consistency. I take a solution of ammonium dichromate (one-half ounce dissolved in cold water to give a fine solution) and stir this 80 into the calcimine cream adding about four quarts of water to bring the whole to a water thin paint consistency adapted to be applied as a paint or coating to the screen. 85

This introduces a binding and a waterproofing factor and gives to the mixture a setting texture that is very highly desirable. One important effect of such a coating lies in its fireproofing or fire retarding effect. The coating is so resistant that if applied 90 even to paper it may be exposed to flame. My coating, therefore, affords for any surface a very considerable flame resistance which in the case of ordinary drops is a 95 most important factor.

In addition to these factors as will be discussed later, I introduce glycerine into the mixture. As explained the usual screen or drop problem is a hard one regarded 100 mechanically. By providing for a maximum of flexibility in my coating I make the treated surface so flexible that it is capable of withstanding extremely rough usages. Moreover, my coating made as indicated is 105 capable of adaptation to, or the filling of defects and blemishes in the screen surface so that they are imperceivable in the picture as projected. These relate to the physical make up of the coating but there remains 110 the important chromatic factor.

For this I prepare a coloring which may be considered in three parts.

- First, I establish a blue which I preferably produce as follows: Taking for convenience one pint flasks I fill to three-quarters with glycerine. In this I dissolve (with heat) my dyes. I prepare three sets of dyes, i. e. blue, Turkey red and green. These dyes obviously vary in color and intensity but for sake of simplicity I refer to well known standard commercial dyes, i. e. take such commercial dyes as Diamond dyes. Of these I take of the blue one commercial package placing it in one of the flasks and agitating. I take one package of the Turkey red and shake into another flask and similarly introduce one package of the green in the third. The uncorked flasks should then be heated in hot water standing for one-half hour. They can then be corked and allowed to stand for thirty-six hours more.
- The resultant glycerine solutions will be clear and complete and in condition for subsequent use. To the mix from the original five pound batch I add of the green solution five drops; of the blue solution twenty drops and of the Turkey red solution one-half ounce. These are added with stirrings maintaining the same direction.
- I add these by consistent stirrings in the same direction until entirely blended but as

they are inferior amounts the predominant whiteness is not visibly altered. The resultant mixture of "paint" may be applied by brush or otherwise to screen or other surfaces or otherwise embodied thereon.

The surface so produced is extremely responsive to the varied qualities of the projected picture. The blue accommodates the blue factor of the picture and at the same time correlates the so-called white of the calcimine. The green is responsive to the green rays of the source of projection while the red is directly responsive to the general red conditions of photographic reproduction.

Various modifications may be resorted to in composition, color relation and other properties such as waterproofing, and all without passing the bounds of my invention.

What I therefore claim and desire to secure by Letters Patent is:

A coating for picture screens and the like comprising finely divided white calcareous base, an ammonium dichromate dissolved therein, and plural elementary dyes introduced therein in amounts insufficient to visibly change the apparent whiteness, but responsive to color in a projected beam.

In testimony whereof I have hereunto affixed my signature.

HENRY E. JODOIN.